

(No Model.)

G. S. LEE.

ROADWAY OR PAVEMENT.

No. 394,583.

Patented Dec. 18, 1888.



*Witnesses.*

*Robert Enrett,*  
*J. A. Rutherford.*

*Inventor:*

*George S. Lee.*  
*By*  
*James L. Norris*  
*Atty.*

# UNITED STATES PATENT OFFICE.

GEORGE S. LEE, OF DENVER, COLORADO, ASSIGNOR TO SAMUEL H. BATES,  
OF SAME PLACE.

## ROADWAY OR PAVEMENT.

SPECIFICATION forming part of Letters Patent No. 394,583, dated December 18, 1888.

Application filed November 22, 1887. Serial No. 255,912. (No model.)

*To all whom it may concern:*

Be it known that I, GEORGE S. LEE, a citizen of the United States, residing at Denver, in the county of Arapahoe and State of Colorado, have invented new and useful Improvements in Roadways or Pavements, of which the following is a specification.

My invention relates to the construction of roadways or pavements; and its object is to 10 furnish a pavement or roadway of smooth surface, yet affording a good firm foothold for animals traveling thereon, economical in construction, yet durable; to which ends it consists in the features more particularly hereinafter described and claimed.

In the construction of my improved roadway I prefer to use the composition of matter described and claimed in my application of even date herewith and bearing Serial No. 20 255,911, which composition consists, essentially, of "iron slag," the refuse or slag from gold and silver reduction-works, and a cementing material, such as asphalt.

Ordinarily in the construction of concrete 25 or asphaltic pavements and roadways the coarser composition—that is, the composition formed of the asphalt or cement and gravel or broken stone of some considerable size, say one or two inches diameter—is placed at 30 the bottom as the lower layer, while the upper layer, upon which comes all the grinding wear, is composed of cement or asphalt and sand or very finely-communited rock material, so that the composition most susceptible to 35 the wear of travel is the one fully exposed thereto. This arises from the fact that the rock or gravel used is always harder than the cement or asphalt matrix in which it is embedded, and consequently wears away more 40 slowly; hence if the coarser composition were used as the top or surface layer the cement or matrix under ordinary conditions would wear away faster than the embedded gravel or rock, either leaving the latter projecting above 45 the general level of the road-bed, making the latter uneven, rough, and uncomfortable, or the gravel or rock would by the concussion of wheels, &c., be loosened from the matrix and removed therefrom, leaving the roadway 50 pitted, the pits speedily enlarging into holes

needling repairs. By the use of the composition noted, however, the coarser and better-wearing material or composition may be used as the surface or wearing layer, inasmuch as the iron slag used—essentially in its composition an "iron glass" formed principally of protoxide of iron and silica—wears equally and evenly with the remainder of the materials used. While very hard it is also brittle, and while the asphalt or matrix is ground 55 away by the action of vehicles passing thereover the slag is also ground away, leaving the surface level and even; at the same time, being used in this surface layer in a coarse form, it preserves a somewhat rough though 60 level surface, affording a good firm foothold.

In laying my improved roadway or pavement, the ground is first leveled and the bed brought to the desired curve or radius. If the bed be on hard or clay soil, the laying may 70 proceed thereon without further preparation than such leveling and proper tamping. If, however, the bed be on sandy or soft soil, it is preferable to "fur" the bed by spreading thereon a layer, a few inches in thickness, of 75 crushed slag, well tamped and compacted. The bed or foundation being thus prepared, the first layer or course is spread thereon, which is formed of the slag referred to, crushed so as to readily pass through a twenty-mesh screen, 80 and which forms about seventy-five per cent. of the bulk of the composition. To this is added about five per cent. each of talc and fire-clay and two per cent. of lime. These ingredients being thoroughly mixed, <sup>there</sup> are added 85 about ten per cent. of crude or commercial asphaltum and two to three per cent. of crude petroleum as the cementing material, the whole being thoroughly mixed and blended together. This layer being well compacted, a 90 second or surface layer is laid thereon, which layer consists of the same ingredients prepared in the same manner, excepting that the slag is broken or crushed much coarser—say of such size as would pass through an inch 95 ring or even larger—so as to place the heavier and better-wearing composition upon the surface. In order to unite the two layers the more thoroughly, and also to render the pavement more firm and to avoid danger of the com- 100

- pound "creeping" from the crown to the edges, especially when considerable curve or radius is given the roadway, timbers may be embedded therein, the timbers being partially  
5 embedded in each layer and totally inclosed by the two layers; and these timbers may themselves be braced by cross-timbers secured thereto on the top or bottom, or both, by braces extending between them.  
10 The construction of this pavement is illustrated in the accompanying drawing, which is a perspective view, partly in section, of my improved pavement.

In the view the reference-numeral 1 indicates the foundation or bed smoothed, compacted, and brought to the proper curve or radius between the sidewalks 8 8. Upon this bed is laid the first layer 2, which is of the finer material, as before described. During the process of laying this layer longitudinally-arranged timbers 4 4 are partially embedded therein at proper intervals, as shown. While these timbers may be of any desired size and at any suitable distances apart, I prefer, as giving very good results, to use timbers either two by four or two by six inches in cross-section, and to place them four to six feet apart.

In order to stiffen and brace these main timbers themselves auxiliary cross-timbers may be used. These may be timbers 6, laid upon the tops of the timbers 4 and transversely thereto, and abutting against a central strip, 8, whereby an elastic support is given to the roadway.

3 3 represent the guttering, which, if of sep-

arate organization—as of iron, tile, or stone—should be laid on layer 2. The upper layer, 7, of the coarser material is then laid from curb to curb or from gutter to gutter, being well tamped into the interstices between the bracing-timbers, the whole being well rolled and compacted in the usual manner. The pavement outside the gutters may be a continuation of the layer 7. These bracing-timbers, it will be seen, are partially embedded in each layer and totally inclosed by the two layers.

Having thus described my invention, what I claim is—

1. A roadway or pavement consisting of two layers of composition composed, essentially, of iron slag from gold and silver reduction works, and a series of longitudinal and transverse timbers embedded in said composition, whereof the upper layer is the coarser, said transverse timbers having their ends abutting against a central longitudinal strip, substantially as described.

2. A roadway or pavement consisting of a series of longitudinal timbers, a series of transverse timbers having their ends abutting against a central strip, and one or more layers of composition covering and inclosing the same, substantially as described.

In testimony whereof I affix my signature in presence of two witnesses.

GEORGE S. LEE.

Witnesses:

JAMES L. NORRIS,  
J. A. RUTHERFORD.